

# UNITED STATES PATENT OFFICE.

RICHARD GEORGE WOODBRIDGE, JR., OF WILMINGTON, DELAWARE, ASSIGNOR TO  
E. I. DU PONT DE NEMOURS & COMPANY, OF WILMINGTON, DELAWARE, A CORPO-  
RATION OF DELAWARE.

## PROCESS OF MAKING PROPELLENT POWDER.

1,396,493.

Specification of Letters Patent.

Patented Nov. 8, 1921.

No Drawing.

Application filed March 14, 1921. Serial No. 452,263.

To all whom it may concern:

Be it known that I, RICHARD GEORGE WOODBRIDGE, Jr., a citizen of the United States, and a resident of Wilmington, in 5 the county of New Castle and State of Delaware, have invented a certain new and useful Process of Making Propellant Powders, of which the following is a specification.

This invention relates to the production 10 of nitrocellulose powders of the progressive type, and comprises treating nitrocellulose powder grains with a deterrent material at an elevated temperature for a sufficient length of time to cause substantial impregnation of said grains by the deterrent material.

Improvements in processes of manufacturing progressive propellant powders have been described by me in Patents 1312463 and 20 1313459. According to the processes set forth in said patents thorough impregnation of nitrocellulose grains with a deterrent material was brought about by subjecting a mixture of the two materials to a prolonged 25 treatment with hot water. Powders made in this manner gave much better ballistic results than powder made by processes known in the prior art, such as the process of British Patent 15553 of 1898 to Frederick 30 William Jones.

Jones was satisfied with obtaining a very superficial impregnation of the surface of the powder grains such as would result from applying to the powder grains and surface 35 coating material, sufficient heat to melt the latter. That in fact Jones made no attempt to secure complete impregnation of the powder grains is made clear in the description of his process set forth in the above mentioned patent; thus, for instance, in lines 10-27 page 5 he says—"When using dinitrotoluene for this purpose, I first crush it to an impalpable powder. I then add it in the powdered form to a charge of the gun- 40 powder in the drum. The proportion of dinitrotoluene added will be considerably greater than the proportion eventually taken up by the gun-powder, and may amount to as much as say, 5 per cent. I then drum 45 the mixture for a period of time, perhaps 8 hours, more or less, which suffices to cause the grains to take up so much of the dinitrotoluene as is desired. I then remove the charge from the drum and sift it in order to

separate the coated gunpowder from the 55 residue of dinitrotoluene. I then take the coated powder and expose it in a suitable oven to a temperature of about 70° C. At this temperature the dinitrotoluene will melt, but being already evenly distributed 60 over the grain, it does not, when brought into the molten condition, penetrate the grain owing to the viscous nature of the solid solvents and the small amount of nitrocellulose dissolved. The dinitrotoluene remains 65 where it has been placed and the only effect of its being brought to the molten condition is that it becomes strongly adherent to the grain forming a non-explosive shell. In all cases, I prefer to glaze the coated grains 70 with graphite to make them smooth and easy to load with."

A slower burning powder is in fact obtained by the Jones process just quoted, but such powder lacks the advantageous ballistic properties which characterize the powders made according to the above mentioned 75 Patents Nos. 1312463 and 1313459.

In a further investigation of this subject to ascertain whether or not it was possible to 80 improve the ballistics of a powder made substantially in accordance with the directions of the Jones patent, I caused a large number of samples of such powder to be maintained for different periods of time, ranging 85 from 15 minutes to 96 hours, at a temperature just sufficient to melt the deterrent material (a temperature of 70° C. when the deterrent was dinitrotoluene). Some remarkable results were obtained from this 90 series of tests. The samples heated for various periods up to two hours showed practically no effect from this treatment, but samples heated for substantially more than two hours were found to have decidedly improved ballistic properties. The extent of 95 the improvement in powders heated for more than two hours is indicated by the decrease in the pressure generated as compared with that generated by powder heated for less 100 than 2 hours, the weights of charges in the different cases being such as to impart to the bullets substantially equal velocities; this decrease in pressure amounted to more than 2000 pounds per square inch.

The tests above mentioned may be described in greater detail as follows:

Smokeless powder was treated with about

5% of its weight of dinitrotoluene exactly in accordance with the directions contained in Jones's British Patent 15553/98 *i. e.*, drumming the mixture of powder and dinitrotoluene for a period of 8 hours, more or less, and then heating the powder thus coated in an oven at 70° C.; but instead of heating only until the coating became molten, the heating was prolonged to the extent hereinafter indicated. The samples of the powder removed after 15 minutes, 1 hour, and two hours, respectively, of heating at 70° C., cooled and glazed with graphite, showed little or no improvement in ballistics except giving a slower burning powder requiring a higher weight of charge to give the same velocity with relatively no increase in pressure. To illustrate this point, I give the following ballistic results obtained in the U. S. 30/06 rifle using a 150-grain bullet:

| Time heating at 70° C. | Weight charge (grains) | Mean instrumental velocity at 78 f. s. | Mean pressure (lbs. per sq. in.) |
|------------------------|------------------------|----------------------------------------|----------------------------------|
| none                   | 40.5                   | 2617                                   | 43320                            |
| 15 min.                | 42.0                   | 2613                                   | 43600                            |
| 1 hour                 | 42.3                   | 2616                                   | 44180                            |
| 2 hours                | 43.2                   | 2643                                   | 43760                            |

This heat treatment was continued, however, at 70° C. up to 96 hours and ballistic tests were made on samples removed after 6, 12, 24, 48, 72, and 96 hours. The results of ballistic tests on powder after 6 hours treatment showed a decided improvement as compared with the powder heated two hours. Furthermore, the tests show that no material improvement is obtained by extending the time of heat treatment at 70° C. beyond the 6 hour period. These results are as follows:—

| Hours heating at 70° C. | Weight charge (grains) | Velocity at 78 ft. per s. | Mean pressure (lbs. per sq. in.) |
|-------------------------|------------------------|---------------------------|----------------------------------|
| 6                       | 43.4                   | 2642                      | 41200                            |
| 12                      | 43.2                   | 2639                      | 41940                            |
| 24                      | 43.2                   | 2628                      | 41400                            |
| 48                      | 43.2                   | 2629                      | 41620                            |
| 72                      | 42.9                   | 2633                      | 41880                            |
| 96                      | 42.9                   | 2620                      | 41340                            |

The above-described experiments showed clearly that no improvement in ballistic results was obtainable in surface coating this particular type of base grain when the dinitrotoluene was left on the surface of the grain as an exterior coating, and that a definite heat treatment at 70° C. was necessary in order to secure that impregnation of the surface of the powder by the dinitrotoluene which would result in giving a powder of improved ballistics. In describing the duration of the heat treatment it may therefore be said, in general, that the heating should be continued until the deterrent material

no longer exists on the surface of the powder grains as a distinct layer. After the heat treatment has been continued for the proper length of time the deterrent is found concentrated near the surface of the powder grains, but it has penetrated into the same for a considerable depth so that in the burning of the powder the successively exposed surfaces contain less and less of the deterrent, thus causing the combustion to proceed with increasing rapidity. Such powders give a lower temperature in the gun, tending to reduce the erosion and flash produced and allow the attainment of a high velocity without undue increase in the pressure. 75 80

The process is applicable to the various kinds of small arms and cannon powders.

In the above description of the new process I have said that the powder, coated with, for example, dinitrotoluene, is heated for substantially more than 2 hours at a temperature of about 70° C. It is desirable, especially when large batches of powder are being treated, to cause the increase in temperature up to the final temperature of 70° C. to take place gradually. The tendency of the powder grains to stick together may be overcome by thoroughly mixing a small percentage of graphite therewith sometime before the temperature has reached the melting point of the deterrent material. 90 95

For the deterrent material I prefer to use 2,4-dinitrotoluene, but the other isomeric dinitrotoluenes or mixtures thereof may also be used, as well as the mononitrotoluenes. 100 Instead of the foregoing explosive deterrents, I may use a mixture containing non-explosive deterrents as, for example, dimethyldiphenylurea and phenylacetanilid. The deterrent material used, whether composed of a single substance or a mixture of substances, should preferably have a softening or melting point of such a value that impregnation of the grains will occur at a temperature of from about 70 to 80° C. 110

In the ordinary practice of the new process the powder, coated with from about 1 to 5% of deterrent material, is heated for the required length of time in the presence of air, but it is to be understood that the powder may alternatively be heated in the presence of any other inert medium as, for instance, carbon dioxide or nitrogen. The essential difference between the present process and the processes described in various prior patents in this particular art is that the powder, according to the present process, is given a prolonged heat treatment in the absence of any substantial amount of water in either the vapor or liquid form. In other words the powder is heated while dry instead of while wet. 115 120 125

My invention is not limited to the details above set forth but may be modified in various ways within the scope of the appended 130

claims without departing from the spirit of the invention.

I claim:—

1. The process which comprises heating substantially dry nitrocellulose powder grains at a temperature of from about 70 to 80° C. in contact with a deterrent material capable of diffusing into said grains at said temperature, and continuing said heating until substantial impregnation of said grains with said deterrent material has occurred.

2. The process which comprises heating substantially dry nitrocellulose powder grains at a temperature of from about 70 to 80° C. for substantially more than 2 hours in contact with a deterrent material capable of diffusing into said grains at said temperatures.

3. The process which comprises heating substantially dry nitrocellulose powder grains having a coating of a deterrent material amounting to from about 1 to 5% of the weight of the nitrocellulose at a temperature of from about 70 to 80° C. until the deterrent material no longer exists as a separate and distinct layer on said grains.

4. The process which comprises heating substantially dry nitrocellulose powder grains having a coating of a dinitrotoluene amounting to from about 1 to 5% of the

weight of the nitrocellulose at a temperature of from about 70 to 80° C. until the dinitrotoluene no longer exists as a separate and distinct layer on said grains.

5. The process which comprises heating, while immersed in an inert gas, nitrocellulose powder grains having a coating of a dinitrotoluene for substantially more than 2 hours at a temperature of about 70° C. to cause the dinitrotoluene to diffuse into the body of the grains.

6. The process which comprises heating, while immersed in an inert gas, nitrocellulose powder grains mixed with graphite and having a coating of a dinitrotoluene for substantially more than 2 hours at a temperature of about 70° C. to cause the dinitrotoluene to diffuse into the body of the grains.

7. The process which comprises heating substantially dry nitrocellulose powder grains having a coating of a dinitrotoluene amounting to about 5% of the nitrocellulose at a temperature of about 70° C. for more than 2 hours and until substantially all of the dinitrotoluene has diffused into the grains.

In testimony whereof I affix my signature.

RICHARD GEORGE WOODBRIDGE, Jr.